

## UNITED STATES PATENT OFFICE

2,322,859

## LUBRICANT

Clarence M. Loane, Hammond, Ind., and James W. Gaynor, Chicago, Ill., assignors to Standard Oil Company, Chicago, Ill., a corporation of Indiana

No Drawing. Application September 20, 1940,  
Serial No. 359,088

7 Claims. (CL 252—47)

This invention relates to lubricants and particularly to improvements in lubricating oil compositions intended for use in internal combustion engines under severe conditions wherein corrosion, piston ring and cylinder wear, carbon, and varnish formation may be encountered.

Straight petroleum lubricants are effective within certain defined limits of engine operating conditions, and when these limits are exceeded, they frequently fail to give the desired performance demanded of them. Since in modern engines, designed to give increased performance, these limits are frequently exceeded, the use of straight mineral oils as lubricants produces undesirable conditions within the engine; thus varnish and carbon formation is excessive, and corrosion of improved hard metal alloy bearings is encountered.

It is the object of the present invention to provide a lubricant for internal combustion engines which will be effective in providing adequate lubrication for such engines.

It is a further object of the invention to provide a lubricant which will not be inducive to the formation of varnish and/or carbon. Another object of the invention is to provide a lubricant which will reduce engine wear and be non-corrosive to bearings. Other objects and advantages of the invention will become apparent as the description thereof proceeds.

We have discovered that an improved lubricant can be obtained by blending a mineral lubricating oil with from about .05% to about 10%, preferably from about 0.5% to about 5%, of a sulfurized fatty material such as sperm oil, lard oil, tallow and the like and from about .05% to about 5%, preferably from about 0.5% to about 2%, of a complex glyceride phosphoric acid ester such as natural and synthetic phosphatides, for example, lecithin, cephalin, and the mixed phosphatides derived from soybean oil or other commercial sources. Also suitable for this purpose are other esters of phosphoric acid, preferably those containing an amine or quaternary ammonium group.

The sulfurized fatty material should contain from about 5% to about 15% sulfur and should be blended with the oil in amounts sufficient to produce a resultant blend containing from about .05% to about 1.0% added sulfur.

The laboratory tests and engine tests have demonstrated that the blend of mineral oil, sulfurized fatty material, such as sulfurized sperm oil, and the glyceride phosphoric acid ester, such

as a commercial lecithin, possesses extremely satisfactory detergent properties and outstanding stability. Tests were made in a standard six cylinder automobile engine operated at 35 brake horsepower at 3,000 R. P. M. and with an oil sump temperature at 285° F. After sixty hours operation under these conditions, the engine as inspected after each test, was given the following visual rating; a substantially "clean" engine being given a rating of 10.

TABLE I

| 15 | OIL                                 | Visual inspection ratings |             |                  |         |
|----|-------------------------------------|---------------------------|-------------|------------------|---------|
|    |                                     | Varnish                   | Ring carbon | Crankcase sludge | Overall |
| 20 | 1 Control                           | 5                         | 5           | 4                | 4.7     |
|    | 2 Control + 1% commercial lecithin  | 8                         | 8           | 10               | 8.3     |
|    | 3 No. 2 + 3% sulfurized sperm oil   | 9                         | 10          | 9                | 9.3     |
|    | 4 Control + 3% sulfurized sperm oil | 6                         | 5           | 6                | 5.8     |

25 The engine tests as summarized in the above tabulation show that the commercial lecithin effected a reduction in the varnish or lacquer-like deposits normally found on piston skirts, valve stems, guides, etc. Lecithin also decreased the amount of sludge formed on the crankshaft cheeks, on the oil screen, in the oil pan, etc. Sulfurized sperm oil when used as the sole compounding agent in concentrations sufficient to give 0.3% added sulfur, lessened by only a small amount varnish forming tendency, ring carbon and crankcase sludge. Commercial lecithin and sulfurized sperm oil in combination effected a great reduction in varnish formation, and practically eliminated crankcase sludge and ring carbon, and rendered excellent all-around performance as gauged by the general cleanliness of the engine.

30 45 In another test the detergency of the compounded oil was evaluated by measuring the accumulation of the deposits on a metal screen used in an oil filter on a tractor engine. The metal screen filter had a spacing of 0.001 inch and the amount of sludge accumulated on the screen was determined after the tractor engine had been operated at 33 brake horsepower at 1,800 R. P. M. for thirty hours. In Table II are 50 tabulated the data obtained in this test.

TABLE II  
DETERGENCY (FILTER DEPOSIT) TESTS  
33 B. H. P. at 1800 R. P. M.—tractor engine  
Metal-screen type filter element 0.001" spacing

| Test Oil                                            | Added sulfur in final blend | Weight of deposit in 30 hrs. |
|-----------------------------------------------------|-----------------------------|------------------------------|
|                                                     | Per cent                    | Grams                        |
| 20 S. A. E. grade oil                               |                             | 25                           |
| 99% 20 S. A. E. grade oil + 1% commercial lecithin  |                             | 3                            |
| 98% 20 S. A. E. grade oil + 2% commercial lecithin  |                             | 3                            |
| 97% 20 S. A. E. grade oil + 3% sulfurized sperm oil | 0.3                         | 20                           |
| 96% 20 S. A. E. grade oil + 1% commercial lecithin  | 0.3                         | 0.5                          |
| 96% 20 S. A. E. grade oil + 3% sulfurized sperm oil |                             |                              |
| 98% 20 S. A. E. grade oil + 1% commercial lecithin  | 0.1                         | 0.5                          |
| 98% 20 S. A. E. grade oil + 1% sulfurized sperm oil |                             |                              |

The above data show that the phosphatides impart readily discernible detergency to the motor oil, whereas sulfurized sperm oil alone does not. The detergency provided by the commercial lecithin and sulfurized sperm oil in combination is superior to that afforded by the commercial lecithin alone.

It is to be understood that modifications and variations falling within the terms and spirit of the appended claims are included within the scope of the invention which is not limited by the various details disclosed and described.

We claim:

1. A lubricant comprising a lubricating oil, from about 0.05% to about 5% of a glyceride phosphoric acid ester and from about 0.05% to about 10% of a sulfurized fatty oil.
2. A lubricant comprising a lubricating oil, from about 0.05% to about 5% of a glyceride phosphoric acid ester and from about 0.5% to about 10% sulfurized sperm oil.
3. A lubricant comprising a lubricating oil, from about 0.05% to about 5% of a phosphatide and from about 0.05% to about 10% of a sulfurized fatty oil.
4. A lubricant comprising a mineral lubricating oil, from about 0.05% to about 5% of a phosphatide and from about 0.05% to about 10% sulfurized sperm oil.
5. A lubricant comprising a mineral lubricating oil, from about 0.05% to about 5% of mixed phosphatides and from about 0.05% to about 10% of a sulfurized fatty oil.
6. A lubricant as described in claim 5 in which the sulfurized fatty oil is sulfurized sperm oil.
7. A lubricant comprising a mineral lubricating oil, about 0.5% to about 2% lecithin and about 0.5% to about 5% sulfurized sperm oil.

CLARENCE M. LOANE.  
JAMES W. GAYNOR.

CERTIFICATE OF CORRECTION.

Patent No. 2,322,859.

June 29, 1943.

CLARENCE M. LOANE, ET AL.

It is hereby certified that error appears in the printed specification of the above numbered patent requiring correction as follows: Page 2, second column, line 8, claim 2, for "0.5%" read --0.05%--; and that the said Letters Patent should be read with this correction therein that the same may conform to the record of the case in the Patent Office.

Signed and sealed this 27th day of July, A. D. 1943.

Henry Van Arsdale,  
(Seal) Acting Commissioner of Patents.